

XR

3,162,603

Unit

1024D

1024D

3,162,603

Patented Dec. 22, 1964

2

3,162,603

## METHOD OF GROWING IRIDIUM SUBSTITUTED SINGLE CRYSTAL USING BISMUTH OXIDE FLUX

Jack A. Kohn, New Shrewsbury, Robert O. Savage, Jr., Neptune City, and Arthur Tauber, Elberon, N.J., assignors to the United States of America as represented by the Secretary of the Army

No Drawing. Filed Feb. 1, 1963, Ser. No. 256,221

4 Claims. (Cl. 252—62.5)

(Granted under Title 35, U.S. Code (1952), sec. 266)

The invention described herein may be manufactured and used by or for the Government for governmental purposes without the payment of any royalty thereon.

This invention relates to a method of growing single crystals of the general formula  $\text{BaFe}_{12-2x}(\text{Ir}_x\text{Me}_x)\text{O}_{19}$  where  $\text{Me}$  is a divalent metal from the group cobalt, nickel, magnesium, manganese, iron, zinc, or copper and where  $x$  is a number from 0 to 0.6.

An object of this invention is to grow single crystals of the above general formula that are mechanically sound, have well developed crystalline faces and are relatively free of microscopic pits and foreign inclusions. Another object is to grow single crystals of the above general formula for use in microwave and millimeter device applications as in isolators, rotators, filters, power limiters, and harmonic generators. A further object is to grow single crystals of the above general formula that can be recovered by a simple chemical treatment. A still further object is to grow such single crystals at a melting temperature sufficiently low to eliminate the problem of the reduction of  $\text{Fe}^{+3}$ , thus improving the electronic properties of the product. A further object is to grow the single crystals at a temperature that greatly reduces the loss of volatile components. Another object is to grow single crystals possessing both axial and planar magnetic

of the device in which it is incorporated; single crystals intrinsically have narrower line widths; (2) several useful properties are observed only in single crystals; single crystals are important as standards by which to evaluate the performance of polycrystalline materials of the same composition.

It has been found that the aforementioned objectives can be attained by a method involving mixing (a) ferric oxide, (b) barium oxide or barium carbonate, (c) an oxide of a divalent metal from the group cobalt, nickel, magnesium, manganese, iron, zinc, or copper, (d) iridium or iridium oxide and (e) bismuth oxide either dry or with a dispersing agent such as water or ethyl acetate, drying the mixture, heating the mixture in a platinum or iridium crucible between 1200 and 1300°C., slowly cooling the melt 1 to 4°C. per hour to 950°C., and removing the crystals from the crucible by leaching with hot dilute nitric acid (10–20% by volume). The single crystals obtained exhibit black very lustrous, well developed crystallographic faces. Individual crystals measure up to  $\frac{1}{4}$  inch on an edge. The crystals possess both axial and planar magnetic anisotropy. The effective axial anisotropy field of the crystals can be varied from 17,000 towards 0 oersteds by controlling the iridium concentration. Crystals can also be grown having an effective planar anisotropy field from near 0 oersteds to at least 22,000 oersteds. These large anisotropy field changes are accompanied by a relatively small decrease in saturation magnetization and Curie temperature. X-ray diffraction powder and single crystal patterns show that these crystals have the ferroxdure ( $\text{BaFe}_{12}\text{O}_{19}$ ) structure and that the cell volume increases with increasing  $x$ .

Some of the single crystals grown according to the method of the invention with the Batch Starting Composition and resulting magnetic properties are listed in the following table.

TABLE  
Preparation and Properties of Single Crystals in the  
System  $\text{BaFe}_{12-2x}\text{Ir}_x\text{Me}_x\text{O}_{19}$

| Actual Chemical Composition                                                 | Batch Starting Composition                                                                                                                | Magnetic Properties                             |                |                            |                 |                               |                                  |
|-----------------------------------------------------------------------------|-------------------------------------------------------------------------------------------------------------------------------------------|-------------------------------------------------|----------------|----------------------------|-----------------|-------------------------------|----------------------------------|
|                                                                             |                                                                                                                                           | Magnetization Units, gauss cm. <sup>3</sup> /g. |                | Magnetic Moment in $\mu_B$ | Curie Temp. °C. | Anisotropy Field in oersteds  | Ferrimag. Line Width in oersteds |
|                                                                             |                                                                                                                                           | Room Temp.                                      | B.P. Liq. Nit. |                            |                 |                               |                                  |
| 1. $\text{BaFe}_{12}\text{O}_{19}$ -----                                    | 2 moles $\text{BaCO}_3$ , 2 moles $\text{ZnO}$ , 6 moles $\text{Fe}_2\text{O}_3$ , 1 mole $\text{Bi}_2\text{O}_3$ in a platinum crucible. | 72                                              | 103            | 20                         | 450             | Axial Anisotropy $H_a=17,000$ | 53 @ 55 KMC.                     |
| 2. $\text{BaFe}_{11.65}\text{Ir}_{0.16}\text{Zn}_{0.16}\text{O}_{19}$ ----- | Same as 1. plus 4 wt. percent $\text{IrO}_2$ in a platinum crucible.                                                                      | 64                                              | 102            | 20.7                       | 362             | Axial Anisotropy 11,500.      |                                  |
| 3. $\text{BaFe}_{10.88}\text{Ir}_{0.8}\text{Zn}_{0.32}\text{O}_{19}$ -----  | Same as 1. performed in a Iridium crucible.                                                                                               | 47                                              | 78             | 18.9                       | 247             | Planar Anisotropy 22,000.     | 1,175 @ 15 KMC.                  |
| 4. $\text{BaFe}_{10.50}\text{Ir}_{0.32}\text{Zn}_{0.52}\text{O}_{19}$ ----- | Same as 1. plus 8.3 wt. percent Iridium metal.                                                                                            | 59                                              | 96             | -----                      | 287             | Planar Anisotropy.            | 105 @ 17 KMC.                    |

anisotropy. A further object is to grow single crystals for use in devices biased to resonance where compounds with planar anisotropy are required as for example, for harmonic generation.

The single crystals prepared by this invention are magnetic oxides of barium, iron, and iridium, and a divalent metal from the group cobalt, nickel, magnesium, manganese, iron, zinc, or copper having properties which make them potentially useful as a magnetic component at microwave frequencies. Single crystals are sought because: (1) The resonance line width of polycrystalline materials is so large as to limit the sensitivity and efficiency

It can be seen from the table that the single crystals prepared by the method of the invention represent an effective anisotropy field range of from 17,000 oersteds axial in the case of ferroxdure ( $\text{BaFe}_{12}\text{O}_{19}$ ) to 22,000 oersteds planar in the case of  $\text{BaFe}_{10.88}\text{Ir}_{0.8}\text{Zn}_{0.32}\text{O}_{19}$ . Thus the method lends itself to the growing of single crystals in which one can control the anisotropy properties.

In the method of the invention, bismuth oxide ( $\text{Bi}_2\text{O}_3$ ) serves as the fluxing agent. The bismuth oxide acts as a solvent for the iridium. As oxidation of iridium metal at the temperatures and times employed is appreciable, the melt may contain iridium oxide or iridium metal.

3162603

-OR 14 262/62.63

It is preferred to use a platinum crucible in carrying out the method as the amount of iridium introduced can then be critically controlled. An excess of up to 50 mole percent iridium is introduced into the initial melt in view of the volatility of the iridium and the competing side reactions occurring during the formation of the single crystals. The amount of the iridium that will go into the single crystal is also determined by such factors as the maximum temperature to which the melt is raised and the cooling rate of the melt. The amount of iridium that can be introduced into the melt is controlled by its solubility in bismuth oxide at a particular temperature.

In the method, the initial mixture may contain from 45.5 to 50.0 mole percent  $\text{Bi}_2\text{O}_3$ , 9.1 to 12.5 mole percent  $\text{BaO}$ , 27.3 to 37.5 mole percent  $\text{Fe}_2\text{O}_3$ , 9.1 to 12.5 mole percent divalent metal from the group cobalt, nickel, magnesium, manganese, iron, zinc, or copper and 0 to 9.1 mole percent iridium.

The foregoing description is to be considered only as illustrative of the invention and not in limitation thereof.

What is claimed is:

1. The method of growing single crystals of the general formula  $\text{BaFe}_{12-2x}(\text{Ir}_x\text{Me}_x)\text{O}_{19}$  where Me is a divalent metal selected from the group consisting of cobalt, nickel, magnesium, manganese, iron, zinc, and copper and where  $x$  is a number from 0.16 to 0.6 said method comprising (1) mixing (a) ferric oxide, (b) barium oxide, (c) an

oxide of a divalent metal taken from the group consisting of cobalt, nickel, magnesium, manganese, iron, zinc, and copper, (d) iridium and (e) bismuth oxide, (2) heating the mixture in a metallic crucible selected from the group consisting of platinum and iridium between 1200 and 1300° C., (3) slowly cooling the melt 1 to 4° C. per hour to 950° C., and (4) removing the crystals from the crucible by leaching with 10-20 percent by volume nitric acid.

10 2. The method according to claim 1 where single crystals of the formula  $\text{BaFe}_{11.66}\text{Ir}_{0.16}\text{Zn}_{0.16}\text{O}_{19}$  are grown.

3. The method according to claim 1 where single crystals of the formula  $\text{BaFe}_{10.80}\text{Ir}_{0.6}\text{Zn}_{0.6}\text{O}_{19}$  are grown.

4. The method according to claim 1 where single crystals of the formula  $\text{BaFe}_{10.96}\text{Ir}_{0.52}\text{Zn}_{0.52}\text{O}_{19}$  are grown.

#### References Cited by the Examiner

#### UNITED STATES PATENTS

20 2,848,310 8/58 Remeika ----- 23-305  
3,079,240 2/63 Remeika ----- 23-305

#### OTHER REFERENCES

Titova: "Growing Monocrystals of Yttrium Ferrite," Soviets Physics, Solid States (1960), pages 1714-15, translated from: Fizika Tverdogo Tela, vol. 1, No. 12.

MAURICE A. BRINDISI, Primary Examiner.